

## UNITED STATES PATENT OFFICE

CHARLES K. HAGUE, OF DETROIT, MICHIGAN, ASSIGNOR TO SUN OIL COMPANY, OF PHILADELPHIA, PENNSYLVANIA, A CORPORATION OF NEW JERSEY

## PROCESS OF COOLING INTERNAL COMBUSTION ENGINES

No Drawing.

Application filed July 18, 1930. Serial No. 469,005.

In the water cooling systems of internal combustion engines, such, for example, as those employed in automobiles, rust forms at certain loci in the circulatory system, dirt 5 and sludge accumulate, rust, particularly from the motor block, is carried to the radiator and clogs or plugs the small water passages, and impurities in the water attack the solder or other binders or welders, the latter 10 action being especially harmful and dangerous. The resultant deterioration shortens the life of a radiator. The extent and rapidity of the corrosion thus produced varies with the character of the water. Thus, wa- 15 ter which is distinctly alkaline or saline promotes rapid corrosion; and in many regions, due to the alkaline or saline character of the water or to its possession of some other chemical characteristics, the deterioration is so 20 rapid as to give rise to serious trouble and materially shorten the life of certain parts and particularly of the radiator. For ex- 25 ample, in the southern part of Florida, where the water is heavily saline, the life of a radi- ator, due to the solder being eaten away, hardly exceeds two months.

The object of the invention is to provide a liquid for use in such cooling systems which will prevent or minimize deterioration of the 30 radiator and other parts with which the water contacts and which, at the same time, will not materially reduce the heat transfer and which will be a solvent for any non-freezing substance, such as alcohol, glycerin 35 or glycol, which may be desirably added thereto in cold weather.

My invention, in its narrower aspect, comprises a process wherein an internal combustion engine is cooled by utilizing, to absorb 40 heat from the engine and to disseminate that heat into the atmosphere, water to which has been added mineral oil and a fatty acid soap derived from mineral oil, the mixture of mineral oil and fatty acid soap being such as 45 to be miscible with water in all proportions. A desirable specific composition comprises from one-third to one part, by weight, of mineral oil and fatty acid soap to 100 parts of water. For example, if the cooling system of an automobile engine requires five to six gal-

lons of water, there may be desirably added thereto from three to five ounces of the mineral oil-fatty acid soap composition.

The protective action of the specified liquid, which could not be forecasted by the known qualities of the composition added to the water, is explainable on the theory that the oil or the mixture of oil and soap forms a protective coating on the walls of the liquid containers which prevents the accumulation 55 thereon of dirt and sludge and thereby prevents rust or corrosion. I do not, however, undertake to specify with certainty the precise action of the composition whereby it produces the specified result, the only demon- 60 strated fact being that the composition does in fact effectually prevent corrosion or at least reduces it to a substantially harmless 65 degree. My tests show, however, that water that has been admitted to an engine that has 70 been so treated is apparently perfectly clear and not an emulsion. From this it seems obvious that the mixture of soap and oil added to the water has been deposited and is no longer carried in suspension, since, if it were, 75 the emulsion or suspension would be slightly milky.

The efficiency in preventing deterioration by the addition to water of the specified composition for a substantial length of time was 80 capable of proof only by tests involving the lapse of such time. Such tests prove that the composition is operative for a period approx- 85 imating two years. It is probable that the effect is substantially permanent, but only ex- 90 periments continued for a considerably longer period can demonstrate that, conclusively. It may be said with certainty, therefore, that the efficiency of the liquid is not measurably reduced after the lapse of at least a year or 95 two, notwithstanding the usual frequent re-plenishment of the water supply to replace losses by evaporation. Since the composition which is added to the water is quite cheap, it may be desirable to drain the sys- 95 tem and add a new volume of the liquid about once a year; or perhaps, out of excess of caution, somewhat more frequently.

If, as I believe, the action of the liquid is due to the formation on the container walls 100

of a protective coating, this coating may be no thicker than about 1/1000 of an inch or even less.

Any substance or compound which is ordinarily added to water to prevent freezing can be added to the liquid which I use, with which such anti-freezing substances or compounds are soluble or miscible to the same degree as with ordinary water.

The composition which I add to water to produce the liquid used in my cooling system may be that produced in the treatment of lubricating oil stock by the addition of sulphuric or other mineral acid, agitation, withdrawal of the acid sludge, addition of caustic soda or other alkali, agitation, and withdrawal of the alkali precipitate or "soda sludge". This soda sludge may be purified, if desired, by the processes described in the Maitland Patents 1,425,882 and 1,425,884, August 16, 1922, and the Hughes Patent No. 1,577,723, March 23, 1926. A typical composition comprises mineral oil, 46%; soap, 11%; petroleum resins, 17.1%; sodium sulphate, 2.3%; water, 23%. The proportions of the above specified ingredients may be regulated as desired by separating the mineral oil as described in the Alleman Patent No. 1,694,463, December 11, 1928, or by separating the mineral oil and the petroleum resins as described in the Alleman Patent No. 1,694,461. A substantial proportion of mineral oil may be added to the foregoing composition or to the fatty acid soap if the latter is separated. When mixed with water, there is formed a milk-white and substantially perfect emulsion.

In place of mineral oil may be substituted any known animal or vegetable oil, and in place of a fatty acid soap derived from mineral oil may be substituted any fatty acid soap; provided, however, that such oil and soap are miscible with water in practicable proportions. Thus, certain known cutting oils may be substituted for the specific composition herein specified. The composition herein specified, however, presents decided advantages over any other composition, and I therefore claim it specifically as well as generically.

The proportions hereinbefore specified are merely illustrative. It is possible to utilize, and obtain, in greater or less degree, the result sought, by using a substantially smaller proportion of mineral oil and fatty acid soap, say as low as one-twentieth or one-tenth of one per cent. So, also, the proportions may substantially exceed one per cent., say two or three per cent., but without corresponding advantage. So far I have found a proportion of from one-half to two-thirds of one per cent. to be satisfactory.

It is preferable, in practicing my process, to first drain the system of such water as it may contain and then introduce the emulsion

of water, oil and fatty acid soap into the system in the usual way, namely, at the inlet at the top of the radiator. The water, as it evaporates, must be, of course, replenished from time to time. Such evaporation of water and repeated addition of fresh water to the cooling system does not affect the efficiency of the composition due, doubtless, to the fact that the oil or fatty acid soap, or, more probably, both, form an adherent protective coating on the walls of parts that would otherwise be subjected to progressive corrosion.

If a coating of rust is already present in the circulatory system, it is advisable, before adding the composition of water, oil and soap, to flush the system with a hot solution of alkali in order to wash away any oxide which is not cemented to the metal. The drain cock of the radiator should be removed in order to afford as large an opening as possible for the passage of the rust flakes. The nozzle of a hose should then be applied to the filler cap of the radiator to allow the full water pressure to wash out the alkali. The system should then be filled with the composition in the same way in which water is ordinarily supplied thereto.

The composition should not be added at the same time alcohol is added, since an alkali soap will be formed that will foam through the overflow pipe of the radiator. If alcohol has been added to the water and the motor has been run a short time, no soap forms.

I have heretofore stated that the use of my process does not interfere with the use of anti-freeze compositions. One unexpected function of my process is that it insures the efficiency of certain anti-freeze compositions, such as glycerin or glycol, in extremely cold weather. It sometimes happens that the addition of glycerin fails to prevent freezing in zero or sub-zero weather. Thus I have found to be due to the fact that oxide in the water raises the cold test. There may be enough oxide present to raise the cold test 10 or 15° F. By the use of my process, the water is free of this oxide and the glycerin has its calculated anti-freeze value.

There may be a slight reduction in the heat transfer rate due to the coating which it is believed is formed on the water-containing walls; but my experiments show that such reduction, if any, cannot exceed ten per cent. of the retardation of heat transfer due to the coating of rust formed in the water chamber of the motor. Practically, therefore, my process accomplishes still another valuable result, namely, a substantial increase in heat transfer above what it otherwise would be in water circulating systems that have been used a comparatively short time.

Having now fully described my invention, what I claim and desire to protect by Letters Patent is:

1. The process of cooling such part of an internal combustion engine as it is desired to cool while minimizing corrosion which comprises circulating, in heat exchange relation with such engine part and the atmosphere, water to which has been added a relatively small proportion of an oil-containing composition which is miscible with water in any proportion forming an emulsion.
- 10 2. The process of cooling such part of an internal combustion engine as it is desired to cool while minimizing corrosion which comprises circulating, in heat exchange relation with such engine part and the atmosphere, water to which has been added a relatively small proportion of a mixture of oil and fatty acid soap which is miscible with water in any proportion forming an emulsion.
- 20 3. The process of cooling such part of an internal combustion engine as it is desired to cool while minimizing corrosion which comprises circulating, in heat exchange relation with such engine part and the atmosphere, water to which has been added a relatively small proportion of a mixture of mineral oil and fatty acid soap which is miscible with water in any proportion.
- 30 4. The process of cooling such part of an internal combustion engine as it is desired to cool while minimizing corrosion which comprises circulating, in heat exchange relation with such engine part and the atmosphere, water to which has been added a relatively small proportion of a mixture of oil and a fatty acid soap derived from mineral oil and which is miscible with water in any proportion forming an emulsion.
- 40 5. The process of cooling such part of an internal combustion engine as it is desired to cool while minimizing corrosion which comprises circulating, in heat exchange relation with such engine part and the atmosphere, water to which has been added a relatively small proportion of a water miscible mixture of mineral oil and a fatty acid soap derived from mineral oil.
- 50 6. The process of cooling such part of an internal combustion engine as it is desired to cool while minimizing corrosion which comprises circulating, in heat exchange relation with such engine part and the atmosphere, water to which has been added from .05 to 3 per cent. of an oil-containing composition which is miscible with water in the specified proportion forming an emulsion.
- 60 7. The process of cooling such part of an internal combustion engine as it is desired to cool while minimizing corrosion which comprises circulating, in heat exchange relation with such engine part and the atmosphere, water to which has been added from .05 to 3 per cent. of a mixture of oil and fatty acid soap which is miscible with water in the specified proportion forming an emulsion.
8. The process of cooling such part of an internal combustion engine as it is desired to cool while minimizing corrosion which comprises circulating, in heat exchange relation with such engine part and the atmosphere, water to which has been added from .05 to 3 per cent. of a mixture of mineral oil and fatty acid soap derived from mineral oil.
- 70 9. The process of cooling such part of an internal combustion engine as it is desired to cool while minimizing corrosion which comprises circulating, in heat exchange relation with such engine part and the atmosphere, water to which has been added from one-third of one per cent. to one per cent. of an oil-containing composition which is miscible with water in the specified proportion forming an emulsion.
- 80 10. The process of cooling such part of an internal combustion engine as it is desired to cool while minimizing corrosion which comprises circulating, in heat exchange relation with such engine part and the atmosphere, water to which has been added from one-third of one per cent. to one per cent. of a mixture of oil and fatty acid soap which is miscible with water forming an emulsion.
- 85 11. The process of cooling such part of an internal combustion engine as it is desired to cool while minimizing corrosion which comprises circulating, in heat exchange relation with such engine part and the atmosphere, water to which has been added from one-third of one per cent. to one per cent. of a mixture of mineral oil and fatty acid soap derived from mineral oil.
- 90 12. The process of protecting the water circulating system of an internal combustion engine against substantial deterioration which comprises applying to the internal metal surfaces of the system an adherent coating comprising mainly mineral oil.
- 95 13. The process of protecting the water circulating system of an internal combustion engine against substantial deterioration which comprises applying to the internal metal surfaces of the system an adherent coating comprising a composition of mineral oil and fatty acid soap.
- 100 14. In testimony of which invention, I have hereunto set my hand, at Detroit, Mich., on this 12 day of July, 1930.
- 105 CHARLES K. HAGUE.
- 110
- 115
- 120
- 125
- 130